

1

2,901,344

## REMOVAL OF IRON FROM ALUMINUM SURFACES

Melvin H. Brown, Allegheny Township, Westmoreland County, Pa., assignor to Aluminum Company of America, Pittsburgh, Pa., a corporation of Pennsylvania

No Drawing. Application February 7, 1958  
Serial No. 713,784

3 Claims. (Cl. 75—97)

This invention relates to, and has as an object, a convenient, economical treatment for surfaces of aluminum articles to remove iron impurities therefrom. As generally used herein, the term "aluminum" includes both aluminum of various grades and aluminum base alloys.

Containers and other articles made of aluminum and aluminum base alloys are widely used in the chemical industries, and generally may be employed without special surface treatment. However, it has been found that iron impurities on the surfaces of such articles are extremely undesirable for certain applications by reason of the effect which the iron may have upon the material contained or contacted, or even upon the resistance to corrosion of the aluminum article itself. For example, a small amount of iron on the surface of the aluminum sometimes has a contaminating effect in that it is found to promote undesired polymerization of certain plastics or to catalyze the decomposition of hydrogen peroxide.

It has now been found that iron impurities may be removed from the surfaces of aluminum and aluminum base alloy articles by a method in which the article is treated with an aqueous solution containing at least 0.1 percent by weight of soluble citrate ion and at least 0.1 percent by weight of soluble nitrate ion, and having a pH below about 2.75. This method is very effective in removing rolled-in iron, or iron left on an aluminum surface after fabrication.

The ions used in the method just described may be introduced as citric and nitric acids, or as soluble salts of these acids, such as sodium, potassium and ammonium citrates and nitrates, or mixtures thereof. Although large concentrations of citrate ion may be employed, it is preferred to use a solution containing less than about 5 percent by weight since amounts in excess of this provide little or no additional benefit and unduly increase the cost of the solution. Similarly, large concentrations of nitrate ion may be employed, but little additional benefit is derived and etching may become significant, especially if the nitrate ion is introduced as the acid. Generally, a solution containing less than about 10 percent by weight and preferably less than about 5 percent by weight of nitrate ion is utilized.

The more acid solutions clean more quickly, although there is an accompanying tendency to etch the metal surface. This etching may be disregarded for some applications; however, where it is significant, it is preferred to employ a solution having a pH above about 1.0. Also from standpoints of handling and disposal, it is generally

2

preferable to use a solution having a pH above about 1.0. As is well known, the pH of the solution may be adjusted by introducing the ions as the acids and neutralizing with a base whose salt is soluble, such as sodium, potassium and ammonium hydroxides.

The surface may be treated with a solution by immersing the entire article in the solution, or by filling the article with the solution, or by running or spraying the solution over the surface, or in any other manner by which the contact may be effected between the solution and the surface. Generally, agitation or movement of the solution relative to the surface of the article shortens the required period of treatment, and spraying has been found preferable for some applications, especially the treatment of large articles, since a small volume of solution may be utilized, relative to the size of the article.

A simple but effective test for the presence of iron impurities on an aluminum surface is the ferroxyl test, wherein the surface is wet with a solution containing 3 percent by weight of potassium ferricyanide and 3 percent by weight of nitric acid. If any iron is present, a blue spot will form within a few seconds. The test solution should be prepared daily since it deteriorates rapidly upon standing. After such a test, the precipitate formed should be removed prior to the treatment of the present invention since it has been found to interfere with the cleaning action. Soap and brushing may be effectively employed to accomplish this removal.

The time of treatment by the method of the invention will vary with the severity of the iron contamination, the composition of the solution and the mode of effecting contact. Treatment times between  $\frac{1}{2}$  and 100 hours are not uncommon; however, treatment times of less than 24 hours are generally sufficient in the treatment of the normally encountered contamination. If the solution is sprayed against the surface, treatment times may often be reduced by as much as 40 to 75 percent over those required in an immersion treatment.

The solutions used in accordance with the present invention are especially adapted for use at room temperature, i.e., ambient temperatures normally prevailing in commercial and industrial atmospheres such as between about 15 and 40° C. However, these solutions may also be employed at elevated temperatures such as 50° C. and 85° C., or above.

Illustrative of the efficacy of the present invention is the following table representing the results obtained in the treatment of prepared test specimens containing embedded iron impurities, the contamination being considerably more severe than would be generally encountered. The specimens were immersed in cleaning solutions constituted in accordance with this invention and which were maintained at room temperature unless otherwise noted. Referring to the specimens, one group was an aluminum base alloy nominally composed of aluminum, 3.5 percent magnesium and 0.25 percent chromium (designated in the table as A); a second group was one of the commercial grades of aluminum containing a minimum of 99.60 percent aluminum and a maximum of 0.04 percent copper and 0.01 percent manganese, the balance of the impurities generally consisting of silicon and iron (designated as B); the third group was an alumi-

num base alloy nominally composed of aluminum and 1.2 percent manganese (designated as C).

face of an aluminum article which comprises treating said surface with an aqueous solution consisting essentially of

Table of examples

| Citrate Ion, Percent by wt. | Nitrate Ion, Percent by wt. | pH   | Metal         | Hrs. to Clean A.v. | Remarks                                                                  |
|-----------------------------|-----------------------------|------|---------------|--------------------|--------------------------------------------------------------------------|
| 0.1                         | 0.2                         | 1.62 | { A<br>B<br>C | 96<br>80<br>48     | Added as citric and nitric acids.                                        |
| 0.37                        | 5.0                         | 0.10 | { B<br>C      | 1.3<br>1.3         | Added as sodium citrate and nitric acid.                                 |
| 5.0                         | 0.38                        | 1.68 | { A<br>B<br>C | 24<br>24<br>24     | Added as citric acid and sodium nitrate.                                 |
| 7.0                         | 7.0                         | 1.75 | { B<br>C      | 32<br>32           | Added as citric acid and nitric acid. pH adjusted with NaOH.             |
| 1.2                         | 1.2                         | 1.75 | { A<br>B<br>C | 80<br>48<br>64     | Added as citric and nitric acids. pH adjusted with ammonium hydroxide.   |
| 1.2                         | 1.2                         | 1.78 | { B<br>C      | 80<br>80           | Added as citric and nitric acids. pH adjusted with potassium hydroxide.  |
| 2.1                         | 2.1                         | 2.69 | { A<br>B<br>C | 40<br>48<br>64     | Added as citric acid and nitric acid. pH adjusted with sodium hydroxide. |
| 1.5                         | 4.0                         | .27  | { B<br>C      | 2<br>5             | Added as citric acid and nitric acid. Adjusted with sodium hydroxide.    |
| 1.0                         | 0.8                         | 2.25 | { A<br>B<br>C | 64<br>48<br>80     | Added as citric acid and sodium nitrate.                                 |
| 0.8                         | 1.0                         | 1.43 | { A<br>B<br>C | 24<br>48<br>64     | Added as sodium citrate and nitric acid.                                 |
| 1.1                         | 0.8                         | 2.25 | { B<br>C      | 72<br>80           | Maintained at 50° C. Added as citric acid and sodium nitrate.            |
| 1.1                         | 0.8                         | 2.25 | { A<br>B<br>C | 96<br>24<br>32     | Maintained at 85° C. Added as citric acid and sodium nitrate.            |

Of the solutions identified in the foregoing table, it is preferred to employ the solution comprised of 0.8 percent by weight of citrate ion and 1.0 percent by weight of nitrate ion, at room temperature; and this solution may conveniently be made up with sodium citrate and nitric acid. In field use, the spray method of treating aluminum surfaces with this solution is recommended.

Having thus described the invention, I claim:

1. The method of removing iron impurities from a surface of an aluminum article which comprises treating said surface with an aqueous solution consisting essentially of at least 0.1 percent by weight of soluble citrate ion and at least 0.1 percent by weight of soluble nitrate ion, and having a pH below about 2.75.
2. The method in accordance with claim 1 wherein said solution is at a temperature between about 15 and 40° C.
3. The method of removing iron impurities from a sur-

35 at least 0.1 percent by weight of soluble citrate ion and at least 0.1 percent by weight of soluble nitrate ion, and having a pH of between about 1.0 and 2.75.

## References Cited in the file of this patent

## UNITED STATES PATENTS

- |           |          |       |               |
|-----------|----------|-------|---------------|
| 2,477,181 | Holman   | ----- | July 26, 1949 |
| 2,671,717 | Ferguson | ----- | Mar. 9, 1954  |
| 2,705,191 | Jumer    | ----- | Mar. 29, 1955 |

## OTHER REFERENCES

Pfizer: Technical Bulletin, Chemicals for Metal Finishing, No. 61. August 1954. Charles Pfizer and Company, Inc., Brooklyn, New York.

Comprehensive Treatise on Organic and Theoretical Chemistry, Mellor; volume 13, pp. 342-346 and 360-361.